

84

F. J. NAPOLITAN.

PLATE FOR USE IN LINING BURGLAR PROOF VAULTS AND SIMILAR PURPOSES.  
APPLICATION FILED AUG. 13, 1921.

1,422,295.

Patented July 11, 1922.

T19



+69  
45

Inventor  
Francis J. Napolitan  
By his Attorney  
A. Parker Smith

## UNITED STATES PATENT OFFICE.

FRANCIS J. NAPOLITAN, OF JERSEY CITY, NEW JERSEY, ASSIGNOR TO AMERICAN  
ABRASIVE METALS COMPANY, A CORPORATION OF NEW YORK.

## PLATE FOR USE IN LINING BURGLAR-PROOF VAULTS AND SIMILAR PURPOSES.

1,422,295.

Specification of Letters Patent.

Patented July 11, 1922.

Application filed August 13, 1921. Serial No. 492,202.

*To all whom it may concern:*

Be it known that I, FRANCIS J. NAPOLITAN, a citizen of the United States of America, residing at Jersey City, county of Hudson, 5 State of New Jersey, with a post-office address at 51 Tonnele Ave., Jersey City, New Jersey, have invented certain new and useful Improvements in Plates for Use in Lining Burglar-Proof Vaults and Similar Purposes, 10 of which the following is a specification.

My invention relates to the production of plates which shall have the highest attainable resistance to the action of an oxy-acetylene burner or similar cutting torch, and at 15 the same time be resistant to cutting tools. Plates of this character are particularly useful in lining bank vaults and safes liable to be attacked by burglars using drills and oxy-acetylene torches in the effort to penetrate 20 to the interior of the structure, but can be employed to advantage in other situations.

I have discovered that purified and fused aluminum oxide, which is almost equal in 25 hardness to the diamond, is the most effective material available for the formation of plates resistant to the action of drills and other cutting tools. Aluminum oxide as heretofore generally used in the arts has been quite impure. A crystalline mass of the 30 material generally known as aluminum oxide is, in reality, an aggregate of aluminum oxide crystals embedded in a matrix of readily fusible and structurally weak impurities, chiefly iron oxide and silica. I 35 have discovered, on investigation, that by chemical and other means, much of the impurities may be removed, and upon subsequent fusing in the electric furnace or other source of great heat, etc., there is produced 40 a much purer aggregate of aluminum oxide crystals without any matrix of diluents. This melts at a temperature of approximately 2050 degrees centigrade, and consequently it is also highly resistant to the action of the 45 oxy-acetylene torch or similar apparatus cutting by the action of heat. The crystals are in rhombohedral form, thus giving it a fairly low possibility of cleavage and considerable structural strength. This fused 50 aluminum oxide is not workable to a degree which would render it possible to make regularly formed plates out of it, and to produce such plates it is necessary to embed in a matrix of cast iron or other metallic material 55 the irregular masses of the fused aluminum

oxide obtained by breaking up the product of the electric furnace.

In the accompanying drawing I have shown in cross section a plate made in accordance with this embodiment of my invention. 60

1 represents the matrix of cast metallic material, and 2, 2 represent masses of fused aluminum oxide cast and embedded therein in the form of graded aggregate, the smaller 65 particules filling the voids between the larger ones sufficiently to make it impossible for a torch flame or drill to pass through the plate without striking one or more of these bodies of fused aluminum oxide. 70

The aluminum oxide is fused, and perhaps re-fused, in an electric furnace so as properly to crystallize it and free it from impurities, and then broken up into smaller masses by hammering or other suitable 75 treatment.

While the fused aluminum oxide masses prepared and employed as above described have the highest possible resistance to cutting tools, they do not present an equally 80 great resistance to an oxy-acetylene cutting torch or similar heat generating apparatus as the fusion point of the aluminum oxide is only about 2050 degrees centigrade.

I have found that the capacity for resisting heat can be much increased by using an artificial spinelle in place of the fused aluminum oxide without, at the same time, materially reducing the hardness. This spinelle is a fused mixture of aluminum oxide and 85 magnesium oxide. On fusing these together and allowing them to crystallize they form an eutectic mixture or solid solution with aluminum oxide in excess, if the purpose is to retain in the compound the high drill 90 resisting property of that component to as great a degree as possible. The excess of aluminum oxide is rejected by the eutectic which forms as a molten mass of the mixture cools, and such excess exists in the solidified 100 state as crystals of more or less pure aluminum oxide between crystals of the spinelle. The magnesium oxide is highly refractory, fusing at about 2800 degrees centigrade, and having other qualities which make it largely 105 immune to the disintegrating action of an oxy-acetylene cutting torch. These qualities are largely impressed on the eutectic mixture. The matrix of pure aluminum oxide retains its hardness and consequent quality 110

of resisting cutting tools and so does the aluminum constituent of the eutectic mixture. Consequently, the masses of spinelle thus formed are superior to the pure aluminum oxide for the combined purposes of my invention.

Having described my invention I claim:

1. As a new article of manufacture a plate for use in forming bank vaults and similar purposes which plate comprises a matrix of cast iron or other metallic material in which are embedded closely packed masses each comprising fused and crystallized aluminum oxide in the form of a graded aggregate.

2. As an article of manufacture a plate 15 for use in forming bank vaults and similar purposes, which plate comprises a matrix of cast metallic material in which are embedded closely packed masses each consisting of a fused and crystallized mixture of magnesium 20 oxide and aluminum oxide with aluminum oxide in excess of that proportion required to form as eutectic with the magnesium oxide.

FRANCIS J. NAPOLITAN.

Witness:

H. E. McGuire.